# EUROPEAN PATENT SPECIFICATION

(11) **EP 0 392 682 B1**
(45) Date of publication and mention of the grant of the patent: **16.08.1995**
(21) Application number: 90303023.7
(22) Date of filing: 21.03.1990
(51) Int. Cl.: C08G 69/50, D21F 3/00, D21F 7/08, D06M 13/12, D06M 101/34

(54) **Paper machine pressing fabrics**
Papiermaschinendrucktücher
Matériaux textiles aptes à presser dans les machines à papier

(30) Priority: 13.04.1989 US 337627
(43) Date of publication of application: 17.10.1990
(73) Proprietor: ALBANY INTERNATIONAL CORP., Albany, New York 12204 (US)
(72) Inventor: Normandin, Lionel, Rensselaer, New York (US)
(74) Representative: Lowther, Deborah Jane

(56) References cited:
- EP-A- 0 159 635
- DE-A- 910 284
- DE-A- 1 419 467
- DE-A- 1 469 347
- US-A- 2 342 823
- US-A- 2 388 676
- US-A- 3 032 441

## Description

This invention relates to paper machine pressing fabrics and has particular reference to paper machine pressing fabrics formed of a polyamide material and having improved longevity and resistance to flattening in the surface layer.

In paper making machines, a slurry of paper making constituents referred to as "furnish" is deposited on a forming fabric or "wire" and the liquid constituent of the furnish is drawn or extracted through the fabric or wire to produce a self-cohesive sheet. This self-cohesive sheet is then passed to a pressing and then a drying section of the paper making machine.

In the pressing section, the paper sheet is transported by a pressing fabric to a pair of rollers where the fabric and the paper sheet pass between the nip of the rollers to dewater by mechanical pressure the paper sheet.

The paper sheet itself may contain other types of chemical finishes and additives and could be, at the same time, subjected to an elevated temperature in order to aid the dewatering. The paper making pressing fabric together with its sheet of paper tends, therefore, to be subjected to immense pressure at elevated temperatures in a rigorous chemical environment. Paper making pressing fabrics are generally produced by needling batt fiber to a woven base fabric. The fabric has multiple functions: first, to support the formed paper sheet through the press section of the machine; secondly, to accept sheet water expressed at each press nip; and last, to impart a finish or surface texture to the paper sheet.

The batt fiber layer constitutes a "cushion" and support for the paper sheet while the woven base provides the primary channels or voids to accept expressed sheet water. The quality of the batt fiber layer and in particular its surface properties and its consistency of surface properties with time, is of extreme importance. As the surface properties of the batt fiber layer deteriorates, so does the quality of the surface of the paper sheet being pressed, as well as, the uniformity of water removal.

In the nip of the press rolls, the batt fibers are bent and deformed under great pressure and at great frequency. Hence the mechanical properties of the batt fiber are of considerable importance in such processes.

Polyamide 6 and polyamide 6,6 have been used extensively in the manufacture of paper machine pressing fabrics. These polymers are readily formable as fibers and their fiber characteristics can be controlled to make acceptable paper making pressing fabrics.

Treatment of polyamide (PA) fibers in general has been proposed, but none have been specifically concerned with the improvement of the mechanical performance of fibers as used in paper machine clothing. Among the prior proposals for the treatment of polyamide fibers are the following:-

United States Patent Specification No. US-A-2,434,247 relates to the modification of synthetic linear polyamides with formaldehyde and an alcohol to obtain a more elastic nylon for woven fabrics.

United States Patent Specification No. US-A-2,430,953 is concerned with producing nylon yarns with a softer hand, better drape, and in addition, a higher melting point, better dye receptivity and increased resistnce to solvents. The polyamide yarns are reacted with formaldehyde at a pH below 3 in alcohol.

United States Patent Specification No. US-A-2,425,334 relates to modification of polyamides with formaldehyde at a pH less than 3 so that they can be cold drawn by no more than 75% of their original lengths.

United States Patent Specification No. US-A-3,276,839 describes a process for finishing and dyeing synthetic nylon textile materials in the presence of phenol and an aliphatic anion-active compound in alkaline medium.

United States Patent Specification No. US-A-3,322,488 refers to sulfomethylated bisphenol-formaldehyde condensation products used as dye resists for synthetic polyamide fibers.

United States Patent Specification No. US-A-2,533,100 relates to a process for treating synthetic linear polyamides with thio derivatives of phenols or their corresponding reduction products.

United States Patent Specification No. US-A-2,388,676 is concerned with improving the light stability of polyamide fibers by forming a catecholaldehyde resin within the nylon.

In each of the above cases the nylon materials exhibit improved properties for use in apparrel or decorative assembly, i.e. use in conditions that will not be subjected to the agressive physical and chemical environment of a paper making machine.

As paper machine technology improves, speeds, operating temperatures and pressures increase with a result that the tendency of existing pressing fabrics to compact and wear is increased. Furthermore, increased degradation with increasing temperature of operation and increasing speed of the machine results in a significantly shorter service life for these fabrics.

US-A-3 032 441 discloses a process for treating an open-weave fabric of, for example, nylon yarns comprising applying a phenolic-aldehyde resin and then an amino-aldehyde resin to the fabric, preferably in amounts of 5 - 10% and 10 - 20%, respectively, before curing the resin coating thereon. The process improves the fabric's dimensional stability, abrasion-resistance and stiffness and may be used to treat a Fourdrinier cloth.

The present applicant has discovered that a paper making pressing fabric using fibers of various polyamides having an increased amine end group concentration can be further processed and modified to produce significantly improved properties.

The present invention provides a polymeric material from the family of polyamides, in which said polymeric material is obtainable by subjecting a polyamide having an amine end group concentration of at least 60 equivalents/10⁶g to a phenol/aldehyde treatment process, the conditions of said treatment process being such that the intrinsic viscosity is increased by at least 4% compared with the intrinsic viscosity of the untreated polyamide. Preferably, the polymeric material has subsequent to said phenol/aldehyde treatment process been exposed to a heat treatment to further increase the intrinsic viscosity by at least 4%. Said polymeric material may be in the form of fibers. The invention further provides a pressing fabric composed of said fibers.

According to the present invention, there is also provided a paper making pressing fabric comprising a fiber layer formed of polymeric fibers, in which said fibers are obtainable from polyamide fibers having an end group concentration such that the amine end group/carboxy end group ratio is greater than 1 by subjecting the polyamide fibers to a phenol/aldehyde treatment process which increases the intrinsic viscosity by at least 4% compared with the intrinsic viscosity of the untreated polyamide fibers.

In one embodiment of the invention, the amine end group concentration of the polyamide fibers before said phenol/aldehyde treatment is at least 60 equivalents/10⁶g. The polyamide may be polyamide 6,6. Where the polyamide is polyamide 6,6, the intrinsic viscosity after the treatment process is preferably not less than 1.3 dl/g. Said fiber layer may be just the surface layer or layers of a batt structure and/or any portion of a batt up to 100% of the batt structure. The fiber layer may be on a base fabric.

In another aspect of the present invention there is provided a method of making a paper making pressing fabric wherein polyamide fibers having an amine end group concentration of at least 60 equivalent/10⁶ gram are subjected to an aldehyde/phenol treatment process in which the fibers are contacted with an aqueous solution of an aldehyde at an elevated temperature and with an aqueous solution of a phenol at an elevated temperature, the treatment process being carried out at a temperature for a time sufficient to impart an increase in intrinsic viscosity of the polyamide of at least 4%, and thereafter forming a layer of said fibers and needling the layer onto a woven base fabric. The fibers may be formed into a batt layer prior to attaching to the base fabric either before or after the aldehyde/phenol treatment process.

Since the woven base fabrics contain yarns of monofilament, multifilament, or spun from staple fibers, that are usually polyamide based, the technology of the present invention can be utilized for these yarn forms since they are also exposed to the heat, pressure and chemical environment already described. Benefits of dimensional stability, strength retention and maintenance of water handling capacity are all vital, and will be improved using yarns prepared by this invention.

Also, while usual manufacturing techniques apply a batt formed of fiber onto a woven base fabric, this should not limit the scope of this invention. Other methods to apply fiber, to anchor the fiber instead of mechanically needling, whether the base is woven or not, or whether there is even a support base should all be considered in producing a pressing fabric.

The word "fiber" should also not be limited in the sense of size dimensions or shape, but be considered a component. In this sense, therefore, for the purposes of this specification, the use of the term "fiber" should also include "yarns".

Phenols which can be used in this process include phenol, pyrocatechol, resorcinol, hydroquinone, pyrogallol and phloroglucinol, as well as, substituted products of the aforementioned compounds provided at least two reactive sites are left open on the aromatic ring. In addition, bisphenols, dihydroxy-naphthalenes and the like could also be utilized.

Aldehydes applicable to this process are formaldehyde, formaldehyde liberating compounds, oxaldehyde, malonaldehyde, succinaldehyde, glutaraldehyde, adipaldehyde, pimelaldehyde, suberaldehyde, azelaldehyde and sebacaldehyde, and the like, as well as their substituted counterparts.

The treated polyamide batt fibers show an increase in intrinsic viscosity up to 25% depending on the phenolic compound and subsequent heat treatment employed. These fibers also exhibit higher wet elongations relative to standard polyamide fibers both before, but especially after the treatment process. There is also a significant improvement in chemical resistance particularly in terms of resistance to degradation of physical properties caused by oxidation by chlorine containing compounds during use on a paper making machine. Fibers also show increased resistance to abrasion resulting from the pressing of papers containing fillers, such as ground calcium carbonate. Such pressing fabrics have exhibited as much as 100% longer lifetime in use, particularly in hostile chemical and mechanically abrasive environments.

Following is a description by way of example only of methods of carrying the invention into effect.

### EXAMPLE 1

Polyamide 6,6 15d staple fiber having an amine end group concentration of 66.4 equivalent/10⁶ gram and an intrinsic viscosity of 1.35 dl/g was subjected to a phenolic treatment process as described below.

The fiber was first immersed in an aqueous bath consisting of 0.5% ethylene diamine and 2.0% formaldehyde at 54°C (130°F) for 30 minutes. After a rinse, the fiber is then subjected to a second aqueous solution of 1.5% resorcinol and 1% formaldehyde at 54°C (130°F) for one hour. Followed by a rinse cycle, the sample was subsequently air dried and heated 10 minutes at 149°C (300°F).

The Table 1 below compares intrinsic viscosities and tensile properties of fiber processed with the above formulation and untreated PA 6,6 fibers having high and low amine end group concentrations. Table 2 includes data describing the properties after exposure to sodium hypochlorite solution in a standard degradation test.

A 6% increase in intrinsic viscosity is observed for the high amine end group fibers after treatment. In addition, these fibers have higher elongations compared to the Control. This higher elongation contributes to the higher Tensile Energy Absorption or "toughness" values. This parameter is important in considering end-use requirements such as resiliency which is an important factor on a paper machine. The treated high amine end group fibers maintain high elongation and tensile energy absorption relative to the control even after exposure to hypochlorite.

### EXAMPLE 2

Additional PA 6,6 fiber samples having low and high amine concentration were treated as described in Example 1 above (designated as "X" treatment) using 1/10 and 1/2 the chemical concentrations. The samples were then subjected to a simulated papermaking test in which they were exposed to repeated compression for a given number cycles and were reviewed and judged on a relative ranking on a scale of 0 to 5.

Examination of Table 3 below shows that the treated high amine end group fibers give superior properties in terms of improved ranking on the simulated papermaking press. According to the table, the lower the ranking the better the results.

### EXAMPLE 3

One field trial was run on the third press position of a paper machine which produces uncoated printing and writing grades of paper, mainly bond and copy papers.

The particular machine has been identified to have extremely high chlorine residuals in their stock water and shower water (in excess of 2.0 ppm).

The standard fabrics have been chemically treated with the best known art to offer a degree of protection to the polyamide fiber in the batt structure. Even so, effective fabric life is less than three weeks, with substantial wear and compaction causing loss of efficient water removal. In extreme cases, fabrics actually tore off the machine due to the degraded state.

At the time of the trial, the previous three fabrics had run 12 days each, one tearing off. The trial fabric structure utilized was composed of 100% of the modified polyamide fiber, with the addition of the special process steps of the invention. Our trial ran 12 days and was scheduled off. The fabric showed no signs of instability and our analysis of the used fabric revealed low weight loss, no fiber fibrillation and fatigue, and little loss to bulk and water handling capacity.

Subsequent fabrics exposed to the invention's process have run as long as 39 days on this position with the fabrics still in a usable physical condition at time of removal. Competitive fabrics have run no longer than 14 days during this time period.

**Table 3**

| Fibers | Treatment | Papermaking Press Ranking (Scale 0-5) 700,000 Cycles |
|---|---|---|
| High amine end group Control | -- | 3.5 |
| High amine end group | 1/10 X | 2.2 |
| High amine end group | 1/2 X | 1.9 |
| High amine end group | X | 1.9 |
| Low amine end group Control | -- | 3.7 |
| Low amine end group | 1/10 X | 3.8 |
| Low amine end group | X | 3.3 |

## Claims

1. A polymeric material from the family of polyamides, characterised in that said polymeric material is obtainable by subjecting a polyamide having an amine end group concentration of at least 60 equivalents/10⁶g to a phenol/aldehyde treatment process, the conditions of said treatment process being such that the intrinsic viscosity is increased by at least 4% compared with the intrinsic viscosity of the untreated polyamide.

2. A polymeric material as claimed in claim 1, which subsequent to said phenol/aldehyde treatment process has been exposed to a heat treatment to further increase the intrinsic viscosity by at least 4%.

3. Fibers formed from the polymeric material as claimed in claim 1 or claim 2.

4. A pressing fabric composed of fibers as claimed in claim 3.

5. A paper making pressing fabric comprising a fiber layer formed of polymeric fibers, characterised in that said fibers are obtainable from polyamide fibers having an end group concentration such that the ratio of the amine end groups/carboxy end groups is greater than 1 by subjecting the polyamide fibers to a phenol/aldehyde treatment which increases the intrinsic viscosity by at least 4% compared with the intrinsic viscosity of the untreated polyamide fibers.

6. A pressing fabric as claimed in claim 5, wherein the amine end group concentration of the polyamide fibers before said phenol/aldehyde treatment is at least 60 equivalents/10⁶g.

7. A pressing fabric as claimed in claim 5, wherein the polyamide is polyamide 6,6.

8. A pressing fabric as claimed in claim 7, wherein the intrinsic viscosity after treatment is not less than 1.3 dl/g.

9. A pressing fabric as claimed in claim 5, in which the fiber layer is on a base fabric.

10. A method of making a paper making pressing fabric wherein polyamide fibers having an amine end group concentration of at least 60 equivalent/10⁶ gram are subjected to an aldehyde/phenol treatment process in which the fibers are contacted with an aqueous solution of aldehyde at an elevated temperature and with an aqueous solution of a phenol at an elevated temperature, the treatments being carried out at a temperature and for a time sufficient to impart an increase in intrinsic viscosity of the polyamide of at least 4%, and thereafter forming a layer of said fibers and needling the layer onto a woven base fabric.

11. A method as claimed in claim 10, wherein the fiber is formed into a batt layer prior to attaching to the base fabric either before or after the aldehyde/phenol treatment.

12. A method as claimed in claim 10, wherein the phenols used in the treatment of the fiber are selected from the group consisting of phenol, pyrocatechol, resorcinol, hydroquinone, pyrogallol and phloroglucinol.

13. A method as claimed in claim 10, wherein the aldehydes used in the process are selected from the group consisting of formaldehyde, formaldehyde liberating compounds, oxaldehyde, malonaldehyde, succinaldehyde, glutaraldehyde, adipaldehyde, pimelaldehyde, suberaldehyde, azelaldehyde and sebacaldehyde.

## Patentansprüche

1. Ein Polymer-Material aus der Familie der Polyamide, dadurch gekennzeichnet, daß das Polymer-Material erhältlich ist, indem man ein Polyamid mit einer Amin-Endgruppenkonzentration von mindestens 60 Äquivalenten/10⁶g einem Phenol/Aldehyd-Behandlungsprozeß unterwirft, wobei die Bedingungen dieses Behandlungsprozesses derart sind, daß die Strukturviskosität um mindestens 4% erhöht wird im Vergleich mit der Strukturviskosität des unbehandelten Polyamids.

2. Ein Polymer-Material nach Anspruch 1, das nach dem Phenol/Aldehyd-Behandlungsprozeß einer Wärmebehandlung unterworfen worden ist, um die Strukturviskosität um mindestens 4% weiter zu erhöhen.

3. Fasern, hergestellt aus dem Polymer-Material nach Anspruch 1 oder Anspruch 2.

4. Ein Pressentuch, hergestellt aus Fasern nach Anspruch 3.

5. Ein Papiermaschinen-Pressentuch, umfassend eine Faserschicht, gebildet aus Polymer-Fasern, dadurch gekennzeichnet, daß die Fasern erhältlich sind aus Polyamid-Fasern mit einer Endgruppenkonzentration derart, daß das Verhältnis der Amin-Endgruppen/Carboxy-Endgruppen größer als 1 ist, indem die Polyamid-Fasern einer Phenol/Aldehyd-Behandlung unterworfen werden, die die Strukturviskosität um mindestens 4% erhöht im Vergleich mit der Strukturviskosität der unbehandelten Polyamid-Fasern.

6. Ein Pressentuch nach Anspruch 5, bei dem die Amin-Endgruppenkonzentration der Polyamid-Fasern vor der Phenol/Aldehyd-Behandlung mindestens 60 Äquivalente/10⁶g beträgt.

7. Ein Pressentuch nach Anspruch 5, bei dem das Polyamid ein 6,6-Polyamid ist.

8. Ein Pressentuch nach Anspruch 7, bei dem die Strukturviskosität nach der Behandlung nicht niedriger liegt als 1,3 dl/g.

9. Ein Pressentuch nach Anspruch 5, bei dem die Faserschicht sich auf einem Basistuch befindet.

10. Ein Verfahren zum Herstellen eines Papiermaschinen-Preßtuchs, bei dem Polyamid-Fasern mit einer Amin-Endgruppenkonzentration von mindestens 60 Äquivalent/10⁶ Gramm einem Aldehyd/Phenol-Behandlungsprozeß unterworfen werden, in welchem die Fasern mit einer wässrigen Lösung von Aldehyd bei einer erhöhten Temperatur kontaktiert werden sowie mit einer wässrigen Lösung von einem Phenol bei einer erhöhten Temperatur, welche Behandlungen bei einer Temperatur und über eine Zeit ausgeführt werden, die hinreicht, um eine Zunahme der Strukturviskosität des Polyamids von mindestens 4% mit sich zu bringen, und danach eine Schicht dieser Fasern gebildet wird und die Lage auf ein gewebtes Basistuch aufgenadelt wird.

11. Ein Verfahren nach Anspruch 10, bei dem die Faser in eine Vlieslage geformt wird, bevor sie an dem Basistuch befestigt wird, entweder vor oder nach der Aldehyd/Phenol-Behandlung.

12. Ein Verfahren nach Anspruch 10, bei dem die Phenole, die bei der Behandlung der Faser verwendet werden, ausgewählt werden aus der Gruppe, bestehend aus Phenol, Pyrocatechol, Resorcin, Hydrochinon, Pyrogallol und Phloroglucin.

13. Ein Verfahren nach Anspruch 10, bei dem die Aldehyde, die in dem Verfahren eingesetzt werden, ausgewählt werden aus der Gruppe, bestehend aus Formaldehyd, Formaldehyd freisetzenden Verbindungen, Oxaldehyd, Malonaldehyd, Succinaldehyd, Glutaraldehyd, Adipaldehyd, Pimelaldehyd, Suberaldehyd, Azelaldehyd und Sebacaldehyd.

## Revendications

1. Matériau polymérique de la famille des polyamides, caractérisé en ce que ledit matériau polymérique peut être obtenu en soumettant un polyamide ayant une concentration en groupes terminaux de type amine d'au moins 60 équivalents/10⁶ g à un procédé de traitement par un phénol/aldéhyde, les conditions dudit procédé de traitement étant telles que la viscosité intrinsèque est augmentée d'au moins 4% par rapport à la viscosité intrinsèque du polyamide non traité.

2. Matériau polymérique selon la revendication 1, qui a été exposé, après ledit procédé de traitement par un phénol/aldéhyde, à un traitement thermique afin d'accroître de nouveau la viscosité intrinsèque d'au moins 4%.

3. Fibres formées à partir du matériau polymérique selon la revendication 1 ou 2.

4. Matériau textile de pressage composé de fibres selon la revendication 3.

5. Matériau textile de pressage permettant de fabriquer du papier comprenant une couche fibreuse formée de fibres polymériques, caractérisé en ce que lesdites fibres peuvent être obtenues à partir de fibres en polyamide ayant une concentration en groupe terminaux telle que le rapport groupes terminaux de type amine/groupes terminaux de type carboxy soit supérieur à 1 en soumettant les fibres de polyamide à un procédé de traitement par un phénol/aldéhyde, lequel augmente la viscosité intrinsèque d'au moins 4% par rapport à la viscosité intrinsèque des fibres de polyamide non traitées.

6. Matériau textile de pressage selon la revendication 5, dans lequel la concentration en groupes terminaux de type amine des fibres de polyamide avant ledit traitement par un phénol/aldéhyde et d'au moins 60 équivalents/10⁶ g.

7. Matériau textile de pressage selon la revendication 5, dans lequel le polyamide est du polyamide 6,6.

8. Matériau textile de pressage selon la revendication 7, dans lequel la viscosité intrinsèque après traitement n'est pas inférieure à 1,3 dl/g.

9. Matériau textile de pressage selon la revendication 5, dans lequel la couche fibreuse se trouve sur un matériau textile de base.

10. Procédé pour préparer un matériau textile de pressage permettant de fabriquer du papier dans lequel les fibres de polyamide ayant une concentration en groupes terminaux de type amine d'au moins 60 équivalents/10⁶ grammes sont soumises à un procédé de traitement par un aldéhyde/phénol dans lequel les fibres sont mises au contact d'une solution aqueuse d'un aldéhyde à une température élevée et d'une solution aqueuse d'un phénol à une température élevée, les traitements étant réalisés à une température et pendant un temps suffisant afin d'augmenter la viscosité intrinsèque du polyamide d'au moins 4%, et ensuite de former une couche desdites fibres et d'aiguilleter la couche sur un matériau textile à base tissé.

11. Procédé selon la revendication 10, dans lequel la fibre est transformée en couche feutrée non structurée avant d'être attachée sur le matériau textile de base, soit avant, soit après le traitement par un aldéhyde/phénol.

12. Procédé selon la revendication 10, dans lequel les phénols utilisés dans le traitement de la fibre sont sélectionnés parmi le groupe consistant en le phénol, le pyrocatéchol, le résorcinol, l'hydroquinone, le pyrrogallol et le phloroglucinol.

13. Procédé selon la revendication 10, dans lequel les aldéhydes utilisés dans le procédé sont sélectionnés parmi le groupe consistant en le formaldéhyde, des composés libérant du formaldéhyde, l'oxaldéhyde, le malonaldéhyde, le succinaldéhyde, le glutaraldéhyde, l'adipaldéhyde, le pimelaldéhyde, le subéraldéhyde, l'azélaldéhyde et le sébacaldéhyde.
